

Patented Feb. 12, 1929.

1,702,155

# UNITED STATES PATENT OFFICE.

NELLE McGHEE CROUCH, OF COLUMBIA, MISSOURI.

## DYE SET.

No Drawing.

Application filed February 9, 1926. Serial No. 87,175.

This invention relates to the process for setting the colors in dyed material such as cloth, garments and the like.

I am aware that sugar of lead or lead acetate has been used in setting colors during the dyeing process as set forth in Patent 355,935, Thomas Halliday, 1887; I am also aware that Epson salts or magnesium chloride has been used to prepare cloth before dyeing as shown in Patent 803,647, William Warr, 1905. In neither of these cases has there been any idea of setting colors in cloth or the like after the dyeing has been accomplished, and while I use both magnesium chloride and lead acetate the object of the invention is to provide a new dye setting process and combination wherein a novel combination may be used to ensure thorough setting of the colors therein.

The combination I use not only includes the two chemicals above mentioned but also includes aluminum acetate which I have found to have a very superior effect especially in this combination. I take for each gallon of water one-third of an ounce of magnesium chloride, one-third of an ounce of aluminum acetate and one-third of an ounce of lead acetate. This amount is sufficient for two pounds of ordinary textile material and for each additional amount of textile material it is obvious that the pro-

portions should be correspondingly increased. The material is first wet in cold water and then placed in the solution, made as above, while stirring, and is let stand for 35 twelve hours. The material is then removed, rinsed in cold water and washed with a mild soap. Preferably the treated material should be dried in the shade. In the case of garments they may be turned wrong side 40 out and dried in the ordinary manner on a line. It is obvious that piece material can be dried on the line in like manner by so folding that the right side is not exposed to the sun's rays. 45

Having thus described the invention, what is claimed as new, is:

1. As a dye setting composition, an aqueous solution containing aluminum acetate, magnesium chloride and lead acetate. 50

2. As a dye setting composition, an aqueous solution containing aluminum acetate, magnesium chloride and lead acetate in equal parts.

3. As a dye setting composition, an aqueous solution containing aluminum acetate, magnesium chloride and lead acetate in equal parts and one-third ounce of each said ingredients to each gallon of water. 55

In testimony whereof I affix my signature.

NELLE McGHEE CROUCH.